

## UNITED STATES PATENT OFFICE

2,079,414

PROCESS FOR PRODUCING ALCOHOLS  
FROM ESTERS OF NONAROMATIC  
CARBOXYLIC ACIDSWilbur A. Lazier, Marshallton, Del., assignor to  
E. I. du Pont de Nemours & Company, Wil-  
mington, Del., a corporation of DelawareNo Drawing. Application August 20, 1932,  
Serial No. 629,754

49 Claims. (Cl. 260—156)

This invention relates to the production of alcohols, and more particularly to the conversion of esters of carboxylic acids to the corresponding alcohols.

5 This application is a continuation in part of my copending application Serial No. 445,224, filed April 17, 1930.

For many years the successful reduction of acids to the corresponding alcohols has depended upon the tedious and expensive treatment of the acid in absolute alcohol solution with metallic sodium, typified in general by the method of Bouveault and Blanc (Chemisches Centralblatt 1904, II, 184; 1905, II, 1700). The advantages accruing from the use of catalytic methods of hydrogenation are manifold and such methods have largely replaced the older chemical methods of reducing unsaturated compounds to the corresponding saturated bodies. Esters of carboxylic acids, however, represent an important class of unsaturated compounds which thus far have not yielded to the known methods of catalytic hydrogenation.

I have made an exhaustive study of the hydrogenation of esters by the prior art methods, including both the ordinary liquid phase static and vapor phase flow processes. I have worked with liquid-containing systems at hydrogen pressures up to 3500 lbs. per sq. in. and temperatures up to 200° C. and have found that practically no hydrogen is absorbed by lactates, valerates, butyrates, or acetates, even when using the most active copper and nickel catalysts available. Again, when the vapor of methyl formate was passed over a copper-copper oxide catalyst together with hydrogen at ordinary pressure and a temperature of 180° C., substantial gaseous decomposition took place with the formation of oxides of carbon, formaldehyde, and formic acid.

40 Methanol was formed only in traces.

The above mentioned experiments, together with many other along the same general line, have finally led to the discovery of a completely successful method of hydrogenating esters. I have found that the hydrogenation of these compounds to produce alcohols is successful only when operating with active hydrogenating catalysts under superatmospheric pressure, at moderately high temperatures, and with an ample supply of hydrogen. For most low boiling esters, such as ethyl acetate, the preferred temperature is in excess of the probable critical temperature of the ester. It follows in these cases that the process may suitably be operated as a vapor phase process.

55 This invention has as an object to provide a

process for the conversion of esters of carboxylic acids, said acids containing more than one carbon atom per carboxyl group, to the corresponding alcohols. A specific object of the present invention resides in the conversion, by hydrogenation, of esters of aliphatic carboxylic acids to the corresponding alcohols. A further object is to provide a process for obtaining the corresponding alcohols from esters of aliphatic acids which contain as substituents aromatic groups. A still further object is to provide an improved hydrogenation process for the production of the rare alcohols from the corresponding esters. It is also an object to catalytically hydrogenate esters of polybasic aliphatic acids and of hydroxy and ketonic acids to the corresponding polyhydric alcohols. Another object is to carry out the above mentioned processes by the use of highly efficient composite hydrogenation catalysts. Other objects will appear hereinafter.

These objects are accomplished by the following invention which, in its general aspects, comprises admixing the ester to be converted with hydrogen, and heating the ester-hydrogen mixture in the presence of and in contact with a hydrogenating catalyst comprising either a single hydrogenating metal or its oxide, or a mixture of reduced hydrogenating metals and their oxides at an elevated temperature and pressure.

In the following examples I have set forth several of the preferred embodiments of my invention, but they are presented for purposes of illustration and not as a limitation:

*Example 1.*—A hydrogenation catalyst is prepared as follows: 23 grams of cadmium nitrate, 24 grams of copper nitrate, and 245 grams of zinc nitrate are dissolved in 500 cc. of water and mixed at ordinary temperature with an equal volume of water containing 126 grams of ammonium bichromate and 75 cc. of 28% ammonium hydroxide. After stirring, the mixture is exactly neutralized with additional ammonium hydroxide and allowed to settle. After several washes by decantation, the precipitate is dried, ignited at 400° C. and compressed into tablets or grains suitable for use in catalytic gas apparatus.

Twenty-five cc. of the mixed chromite catalyst prepared as above is loaded into an alloy steel reaction vessel capable of being heated and withstanding high pressures. The tube is fitted with a preheater, a pump for injecting liquid ester at a constant rate, a T-connection for introducing hydrogen under pressure, a suitable condenser and trap for separating liquid products, and exit control valves.

The catalyst is heated to and maintained at 370° C. The hydrogen pressure is allowed to build up to 3200 lbs. per square inch and under these conditions a mixture of 175 cc. of liquid 5 ethyl acetate and 300 liters of hydrogen, measured at ordinary conditions of temperature and pressure, are passed through the reaction system per hour. With good cooling, the liquid products nearly equal in volume the ester pumped 10 into the system. By determination of the saponification value of the condensate and by distillation analysis, it is found that 75% of the ethyl acetate has been converted into ethanol.

When the process just described is carried out 15 at a slightly higher temperature and a lower space velocity, partial condensation of the reduction products takes place with the formation of a higher alcohol. Thus, butanol is formed from ethyl acetate in substantial yields, in addition to ethanol. For example, when ethyl acetate was passed over the catalyst at the rate of 20 50 cc. per hour under the conditions given in the above example, the condensate contained 26.6% of saturated oily products consisting al- 25 most entirely of butanol and higher alcohols. As the rate of flow of the ethyl acetate is increased, the formation of higher alcohols by con- densation decreases.

*Example 2.*—A copper catalyst is prepared by 30 fusing 8 parts by weight of pure copper oxide with one part of zinc oxide and one part of magnesium oxide. The cooled mass is crushed, screened, and reduced at 150° C. in a stream of diluted hydrogen containing 80% carbon di- 35 oxide and 20% hydrogen. Ethyl n-butyrate is pumped over 25 cc. of catalyst at the rate of 220 cc. of liquid ester per hour, together with hydrogen at the rate of 385 liters per hour, giving a hydrogen-ester molecular ratio of about 40 10 to 1, while the temperature is maintained at 322° C. and the pressure at 2680 lbs. per square inch. By distillation of one liter of condensate, there is obtained about 440 grams of unchanged ethyl n-butyrate, about 270 grams of n-butyl 45 alcohol and about 160 grams of ethanol, representing in all a conversion of about 50% of the ester to alcohol.

*Example 3.*—N-butyl acetate is hydrogenated by passing it, together with hydrogen, over a 50 catalyst prepared as described in Example 1. At a temperature of 350° C. and a pressure of 3000 lbs. there is formed an equimolecular mixture of ethanol and n-butanol representing a conversion of the ester of about 60% when 8 parts 55 of liquid n-butyl acetate by volume is passed over one part by volume of catalyst per hour with a hydrogen-ester molecular ratio of 10 to 1.

*Example 4.*—A copper chromite catalyst is prepared by igniting copper ammonium chromate to 60 its decomposition temperature. The catalyst may be reduced in a stream of hydrogen prior to its use or it may be employed directly, reduction in this case taking place in the presence of hydrogen during the reaction. Two hundred cc. of liquid 65 n-butyl acetate and 260-300 liters of hydrogen are passed over 25 cc. of the catalyst per hour at a temperature of 325° C. and at a pressure of 2600-3200 lbs. per square inch. The effluent condensate contains about 64 grams of un- 70 converted n-butyl acetate per 100 cc. introduced, indicating a conversion to an equimolecular mixture of ethanol and butanol of about 20%.

*Example 5.*—A catalyst prepared as described in Example 1 is heated to 365° C. A mixture of 75 ethyl laurate vapor and hydrogen in the molecular

ratio of 1 to 16 is passed over the catalyst at a pressure of 3100 lbs. High conversions are obtained by pumping the hydrogen-ester mixture over the catalyst at the rate of about 200 cc. of liquid ester per hour per 25 cc. of catalyst. Upon chilling the condensate as thus obtained solid lauryl alcohol may be separated. Six hundred eighty cc. of condensate obtained from 740 cc. of ethyl laurate on distillation yielded 450 grams of pure lauryl alcohol, representing a conversion of 80%. 10

*Example 6.*—Ethyl phenylacetate was vaporized and passed over 25 cc. of catalyst prepared as described in Example 1 at the rate of 285 cc. of liquid ester per hour, together with 420 liters of hydrogen per hour, giving an ester-alcohol molecular ratio of about 10. The pressure was 3000 lbs. and the temperature was maintained at 350° C. The difference in saponification value of the ester before and after treatment indicated a conversion of 92%. From 105 cc. of liquid 20 ethyl phenylacetate passed over the catalyst there was obtained by vacuum distillation 90 cc. of phenylethyl alcohol, together with a little styrene. 15

*Example 7.*—A sample of 93% n-butyl n-butyrate was subjected to hydrogenation over the catalyst of Example 1. The rate of flow was 700 cc. of ester per 100 cc. of catalyst per hour. The system was heated to 346° C. and maintained at a pressure of 2600-3200 lbs. The hydrogen-ester molecular ratio was 13.8. From 710 cc. of the butyrate so treated there was obtained by distillation 580 cc. of pure n-butanol boiling at 117° C., representing a conversion of the ester to butanol of approximately 73% of the theoretical. 30

*Example 8.*—Twenty-five cc. of a catalyst prepared as in Example 1 was loaded into a converter and heated to a temperature of 380° C. in a stream of hydrogen. The pressure was maintained at 3000 lbs. per square inch while a mixture of hydrogen and ethyl acetate vapor was pumped over the catalyst for 2.5 hours in order to obtain steady operating conditions. Without interrupting the flow or changing the conditions of temperature or pressure, the pump was switched from ethyl acetate to a supply of ethyl adipate (the diethyl ester of adipic acid). Seven hundred and fifty five cc. of this ester was pumped through the reaction system in three 50 hours, during which time the volume of hydrogen, measured at ordinary conditions of temperature and pressure, passed through the catalyst was 560 liters. By cooling the exit vapors, there was obtained 736 cc. of liquid products. A 55 comparison of the saponification values before and after treatment showed that the ester content had dropped about 53%. By careful vacuum distillation, there was obtained 210 grams of hexamethylene glycol boiling at 143-144° C. at 60 a pressure of 4 mm. This value corresponds to 48% of the glycol theoretically obtainable from the volume of diethyl adipate treated. 45

The hydrogenation of ethyl adipate at slightly higher temperatures and lower rates of flow 65 than those specified in the above example results in the formation of secondary hydrogenation products consisting of one or more monohydric alcohols.

*Example 9.*—Fifteen hundred grams of copper 70 nitrate dissolved in 4 liters of water was mixed with a solution containing 1000 grams of ammonium chromate in an equal volume of water. Ammonium hydroxide was added to neutralize the acidity developed during precipitation of the 75

copper ammonium chromate. The precipitate was washed by decantation, filtered, and dried, after which it was ignited at a temperature to 400° C. The resulting copper chromite powder 5 was employed for the hydrogenation of esters without further treatment. One hundred fifty grams of ethyl azelate and 15 grams of copper chromite, prepared as described, were placed in a shaking autoclave. Hydrogen was introduced 10 until the pressure reached 3000 pounds per square inch. The mixture was heated to 270° C. and agitated for four hours, after which the absorption of hydrogen had ceased. On recovery and separation of the products, it was 15 found that the yield of nonamethylene glycol was approximately 50%.

In another experiment carried out under approximately the same conditions except that the temperature was raised to 325° ethyl sebacate 20 was hydrogenated in good yields to ethanol and decamethylene glycol. Good results were also obtained by the use of butanol as a diluent for the esters in this process.

*Example 10.*—Copper chromite prepared as 25 described in Example 9 was extracted with 10% acetic acid, washed and dried. One hundred fifty grams of ethyl oleate and 20 grams of the extracted copper chromite were agitated in a shaking autoclave at 250° C. and under a hydrogen pressure of 4900 lbs. After two hours treatment in this manner it was found that the ester had been converted in 83% yields to ethyl alcohol and a mixture of oleyl and stearyl alcohols.

*Example 11.*—The applicability of the process to the production of dihydric alcohols from the esters of certain hydroxy acids is aptly illustrated by an experimental run carried out with ethyl ricinoleate. This ester was passed with 30 hydrogen over 25 cc. of the catalyst described in Example 1 at the rate of about 200 cc. per hour. The average pressure was 2570 lbs. per square inch, the average temperature 370° C., and the rate of hydrogen flow 7.7 cu. ft. per hour. The 35 saponification value of the condensed product indicated a conversion to alcohols amounting to about 65%. In order to remove the remaining olefinic unsaturation, the products were subjected to a further hydrogenation with a nickel catalyst in the liquid phase at 100° C. After distilling off the ethyl alcohol there remained a white solid material consisting of about equal parts of octadecanediol and stearyl alcohol together with a lesser amount of the esters of 40 these alcohols.

*Example 12.*—The diethyl ester of succinic acid was vaporized and passed over the catalyst described in Example 1 together with hydrogen at the rate of 8 volumes of the liquid ester per 45 unit volume of catalyst per hour at a temperature of 367° C. and a pressure of 2500 lbs. per square inch. The hydrogen-ester molecular ratio was about 10. Analysis of the condensed products showed that the ester had been hydrogenated to the extent of about 75%, the principal products being tetramethylene glycol and tetrahydrofuran.

*Example 13.*—Twenty-six g. of barium nitrate and 218 g. of cupric nitrate are dissolved in 50 800 cc. of water by heating to 70°. A solution of 126 g. of ammonium bichromate and 150 cc. of 55 28% ammonium hydroxide in 600 cc. of water is added with stirring. The precipitate is filtered, 60 dried and ignited at 400°. The ignition residue 65

is then extracted twice with 10% acetic acid, washed and dried.

In an alloy steel tube having a capacity of about 400 cc. is placed 252 g. (1.25 moles) of diethyl adipate (b. p. 144—145°/29 mm.) and 20 5 g. of copper chromite catalyst prepared as described above. The tube is closed, made gas-tight, and secured in a suitable agitating device. Connection is made with the hydrogen supply and hydrogen is introduced until a pressure of 10 about 2000 lbs. per square inch is reached. Agitation is started and the reaction system is heated as rapidly as possible to 255° C. Additional hydrogen is now admitted to a total pressure of 15 2000 lbs. per square inch. The temperature is 15 maintained at 255° C. while hydrogen is introduced periodically to maintain the pressure between 2500 and 3000 lbs. After 2-2.5 hours, the rate of absorption of hydrogen becomes quite slow. At this point the temperature is decreased 20 to 240° C. and the hydrogenation is continued until hydrogen absorption is complete. The agitation is stopped and the tube closed off, cooled, and the pressure released. The contents are 25 transferred to a 600 cc. beaker with the aid of four 25 cc. portions of 95% alcohol. The catalyst is removed by filtering with suction and is washed on the filter with four more 25 cc. portions of alcohol. Fifty cc. of 40% sodium hydroxide is added and the alcoholic solution is 30 boiled for 2 hours under a reflux condenser. The solvent is distilled off up to a temperature of 95°. The residue is then transferred to an apparatus for the continuous extraction of liquids 35 and is exhaustively extracted with ether. The ether is distilled and after the removal of water and alcohol the glycol is distilled under vacuum in a 250 cc. Claisen flask. The yield is 125 to 132 g., or 85 to 90% of the theoretical amount. Hexamethylene glycol boils at 143-144° (bath 40 at 160°) under 4 mm. pressure and melts at 41-42°.

Although certain definite conditions of operation, such as temperature, pressure, and rate of flow of the material to be treated over the catalyst, 45 have been indicated in the above examples, it will be apparent that these factors may be varied within wide limits within the scope of my invention. The catalytic reduction of carboxylic esters to alcohols requires the use of temperatures and 50 pressures appreciably higher than customarily employed for other hydrogenation reactions. The temperature may range from about 200° C. up to 500° C. In general the preferred temperature range is 240-400° C., depending somewhat on 55 the catalyst composition selected and the method used for carrying out a given reaction. In operating in the vapor phase it is preferred to use temperatures within the range of 300° C. to 400° C. The success of the process also depends on the 60 use of an elevated pressure in excess of 25 atmospheres, while the preferred pressure is about 50-250 atmospheres per square inch. The maximum pressure which can be used is limited only by the strength of the reaction apparatus. It is 65 to be understood that my invention is not limited to the use of these specific pressures, since they may be varied depending upon the ester treated and the amount of conversion desired. As the pressure is decreased, it will be evident that the 70 conversion to alcohol will decrease in accordance with the well known law of mass action.

In the selection of suitable conditions of temperature and pressure, it is well to remember that the catalytic hydrogenation of esters is a re- 75

- versible reaction that can not be carried to completion in either direction. The best conversions to alcohols are obtained at the highest pressures obtainable in the available equipment and at the lowest temperatures consistent with obtaining a practical rate of reaction. In carrying out the hydrogenation of diethyl adipate as described in Example 13, wherein the liquid phase method was used, it was found that the end products of the reaction at 265° contained about 12% of residual ester whereas at 240° there remained only about 4% of unreduced ester. The advantages of both the higher catalyst activity at the higher temperatures and the low ester content of the equilibrium mixtures at low temperatures may be obtained by carrying out the greater part of the hydrogenation at a moderately high temperature, followed by heating for a limited period at a lower temperature.
- 20 In carrying out the hydrogenation of esters in a continuous reaction system the rate at which the ester may be pumped over the catalyst is a function of the catalytic activity and also of the molecular weight of the ester. An active hydrogenating catalyst will ordinarily convert 8 times its volume of ester per hour. Higher rates of flow of the ester may be employed at the expense of slightly lower conversions. As stated above, particularly in Examples 1 and 8, a lower rate of flow results in a more substantial condensation of the reaction products to yield higher alcohols. The desired rate of flow can be determined by an economic balance between the yields of the different reaction products.
- 35 The ratio of hydrogen to ester used may also be varied over a wide range, but I prefer to use an excess of hydrogen preferably about 5 to 10 moles of hydrogen per mole of ester for most conversions. Whereas the critical factors in the hydrogenation of carboxylic esters are the use of high temperatures and high pressures, it follows that suitable catalysts may consist of any hydrogenating metal or metallic oxide. Catalysts found suitable for the synthesis of methanol from water gas are, in general, also suitable for the hydrogenation of carboxylic esters. For example, I may use reduced metals such as silver, copper, tin, cadmium and lead, and in certain cases iron, cobalt, or nickel. Good results are obtained with fused copper oxide, either wholly or partially reduced. The copper catalyst may be promoted with oxide promoters such as manganese oxide, zinc oxide, magnesium oxide or chromium oxide. These promoted catalysts may be physical mixtures or chemical compounds containing copper, e. g., copper chromate or chromite. A metallic catalyst in the form of a powder may also be used, in which case it is advisable to employ a suitable supporting material such as silica, activated carbon, alumina, or a naturally occurring earth such as kieselguhr. It has been found that elementary nickel supported on kieselguhr and prepared by reduction of the hydroxide or carbonate may be used for the hydrogenation of certain esters, provided a sufficiently high temperature and pressure are used. Such a catalyst, however, has the disadvantage that it has a tendency to carry the hydrogenation completely to hydrocarbons rather than to the more desirable alcoholic intermediate compounds.
- 70 Certain metallic oxides belonging to the class known as difficultly reducible oxides and having both hydrogenating and dehydrogenating propensities may be employed. By the term difficultly reducible is meant that the oxides are not substantially reduced to metal by prolonged exposure

in a state of purity to the action of hydrogen at atmospheric pressure and at a temperature of 400-450° C. Such oxides suitable for the hydrogenation of esters are zinc oxide, manganese oxide, magnesium oxide, etc. These oxides may be employed either alone or in combination with each other or with other oxides which have a promoting action. Preferably the oxide employed as a promoter for the hydrogenating oxide has little activity of itself or is much less active than the hydrogenating oxide employed with it, but it yet serves to further promote the activity of the more active oxide.

It will be noted that the hydrogenating oxides are, in general, of a basic character. The promoting oxides are preferably chosen from the group consisting of the more acidic oxides of elements selected from the higher groups of the Periodic Table. For example, the oxides of chromium, vanadium, tungsten, titanium, and molybdenum are suitable promoters for zinc oxides or manganese oxide. Of these, chromium oxide is preferred, since it inhibits more the tendency towards catalyzing destructive side reactions. I have found it advantageous to use chromium oxide in physical admixture or in chemical combination, e. g., as a chromate or chromite, with a large number of oxides ordinarily regarded as easily reducible. The acidic promoting oxides other than chromium oxide may also be used either in physical admixture or in chemical combination, e. g., as tungstates, vanadates, molybdates, etc. The reducible oxides when combined or otherwise associated with chromium oxides are only partially reduced under conditions of operation and are found to be very effective catalysts for the hydrogenation of esters. The oxides of cadmium, copper, tin, and bismuth are all examples of oxides that may be employed in the more difficultly reducible form. Catalysts consisting of both reduced metals and non-reduced oxides are active even though the reaction is carried out at a temperature above the fusion point of the metal. Such mixed catalysts are conveniently employed initially in the form of chromates or chromites of the metals. Basic zinc chromate when partially reduced with hydrogen is a suitable catalyst for the hydrogenation of esters by virtue of its high activity and absence of side reactions. It may be prepared by treating zinc oxide with chromic acid, by precipitation of the zinc salt with an alkali chromate or by any other suitable means. Manganese oxide-chromium oxide mixtures are also suitable as well as copper oxide in combination with chromium oxide or other acidic oxides.

In carrying out the hydrogenation of esters, I may use any one of the catalysts previously disclosed in my co-pending application No. 285,501, filed June 14, 1928, which has issued as U. S. Patent No. 1,857,921. These catalysts are included among those outlined in the preceding paragraph. A preferred catalyst containing a single hydrogenating metal oxide may be prepared according to the general method described in U. S. Patents 1,746,782 and 1,746,783 and illustrated more fully in Example 1 above. This latter type of catalyst is prepared by ignition of a hydrogenating metal chromate, or of a hydrogenating metal ammonium chromate, or it may be prepared by reduction by hydrogen of the said chromates at a temperature of 500° C. or higher. Particularly good results have been obtained in ester hydrogenation by preparing a catalyst according to the method of U. S. Patent 75

1,746,783 wherein a double ammonium chromate of a hydrogenating metal is heated at about 600° C. to form a chromite catalyst. As indicated in the examples success has attended the use of mixtures of the chromites of two or more hydrogenating metals. The multiple chromite catalyst compositions described in the examples and disclosed in my copending application Serial No. 470,238, filed July 23, 1930, are eminently suited to use in the present invention. The multiple chromite catalyst compositions described in the said copending application may be prepared by precipitation of a mixture of chromates from solution by adding an alkali metal chromite to an aqueous solution of a mixture of hydrogenating metal salts, followed by ignition or by high temperature treatment with hydrogen. I prefer to use a chromite composition consisting substantially of zinc chromite but containing lesser quantities of the chromates or chromites of copper and cadmium. The activity of chromite catalysts may be further enhanced by subjecting the ignited chromites to an acid extraction process which serves to remove from the composition a portion of the hydrogenating metallic oxide which is not combined with the promoter oxide.

The advantages attending the use of difficultly reducible oxides or reducible oxides in a difficultly reducible form are several and substantial. These catalysts possess a high activity and are sturdy in character. They are relatively immune to degenerative processes such as sintering or poisoning, being thus distinguished from metal catalysts which deteriorate rapidly when subjected to excessive heating. Unlike certain metal catalysts, they possess a small tendency to carry the hydrogenation beyond the alcohol stage, for example to the production of the corresponding hydrocarbon.

I wish to make mention of the utility of catalysts containing copper oxide promoted by chromium oxide either in physical mixture or in chemical combination as copper chromate or copper chromite. This catalyst is particularly useful for liquid phase ester hydrogenation reactions.

The catalysts described above, in addition to the modified copper-chromium catalysts last mentioned, may be modified or promoted by the addition of oxides or carbonates of alkali metals or of alkaline earth metals, or of basic compounds of alkali metals or of alkaline earth metals, that is, compounds of these alkali-forming metals with acids which are weaker than the metal hydroxide. Other suitable promoters are compounds containing an alkali or alkaline earth metal combined with the acid radical of an oxygen-containing acid, e. g., barium chromate. These compounds will all be classified under the term "basic compounds of alkali-forming metals". One tendency of the basic promoter is to suppress the further hydrogenation to hydrocarbon of the formed alcohol.

It will be apparent from the above examples that the method of the present invention is applicable in general to the hydrogenation of esters of non-aromatic, i. e., aliphatic and alicyclic carboxylic acids having more than one carbon atom per carboxyl group, but it may be used with particular advantage for the hydrogenation of the esters of non-aromatic monobasic acids to the corresponding monohydric alcohols. Typical acids of this class are acetic, propionic, butyric, caprylic, lauric, capric, myristic, palmitic, linoleic, linolenic, oleic, ricinoleic, stearic, hexahy-

drobenzoic and hexahydrotoluic acids. The process is also valuable for the hydrogenation of esters of non-aromatic dibasic and other polybasic acids to the corresponding glycols and other polyhydric alcohols. Such acids are: hexahydrophtalic, azelaic, sebacic, succinic, suberic, pimelic, nonanedicarboxylic, decamethylenedicarboxylic, brassyllic, dodecamethylene dicarboxylic, hexadecamethylenedicarboxylic, and adipic. The process is also applicable to the hydrogenation of esters of aralkyl acids, which are a species under the class aliphatic acids. Thus, the process is applicable to the esters of such acids as, phenylacetic, phenylpropionic, cinnamic, etc. The hydrogenation of ethyl phenylacetate is described in Example 6 above. The process is also applied effectively to the hydrogenation of esters of hydroxy, aldehydic, and ketonic acids, e. g., lactic, ricinoleic, tartaric, and pyruvic acids, yielding thereby various useful glycols. The process is also applicable to the treatment of mixtures of esters, for example, to the ethyl esters of the mixed acids obtained by the saponification of a fat such as coconut oil, the mixed acids being esterified with ethyl alcohol without separation into the individual components of the mixture. Included within the scope of the invention is the hydrogenation of esters of hydroaromatic acids, e. g., the naphthenic acids, which are included under the term "esters of non-aromatic acids". By the term "esters of non-aromatic carboxylic acids", as used herein and in the claims, I mean to include only esters of acids of the various classes enumerated above. Among the esters to which the present process is applied are the esters of glycerol, glycol and other polyhydric alcohols and mono- and polyesters of the acids named above.

The process is applicable to the type of esters commonly known as waxes, either synthetic or naturally occurring, which on hydrolysis yield high molecular weight aliphatic carboxylic acids and high molecular weight alcohols, e. g., beeswax, spermaceti, carnauba wax and the like. Where the ester is an ester of a polyhydric alcohol it may be a mono ester or a poly ester. Where the ester is an ester of a polycarboxylic acid, it may likewise be a mono ester or a di ester.

The process of my invention also finds application in the conversion of an acid to the corresponding alcohol. I prefer to first form the ethyl ester of the acid in question and subject this compound to hydrogenation in the presence of composite hydrogenating catalysts. In this manner the ethyl alcohol originally employed may be recovered for reacting with a fresh portion of the acid. Methyl alcohol is not as valuable for this purpose, since it is subject to gaseous decomposition during the hydrogenation process. Alcohols such as butanol and propanol may be used successfully when combined as esters with the acids to be reduced.

Aliphatic acids and their derivatives occur in abundance in nature, while the corresponding alcohols are found rarely, if at all. By application of the process of my invention, it is now possible to prepare alcohols from the corresponding acids by first converting these acids to their alkyl esters and hydrogenating the esters under pressure. The usual chemical reducing agents are expensive and have rendered the cost of producing rare alcohols impractical, but by the use of the present invention this obstacle has been

removed, thereby widening the use of these comparatively rare materials in the arts.

The above detailed description contains no specific mention of the hydrogenation of esters of aromatic acids. However, if aromatic acid esters are subjected to hydrogenation under the conditions relating to temperature, pressure, catalysts, etc., described above with respect to aliphatic and hydroaromatic acid esters, hydrogenation will take place, the ester however being preferentially reduced to a hydrocarbon instead of an alcohol. Thus the hydrogenation of ethyl benzoate yields toluene and ethyl alcohol while benzyl benzoate, under the same conditions yields toluene. The broadest scope of the invention therefore is intended to include the hydrogenation of aromatic acid esters although the preferred form relates to the hydrogenation of esters of non-aromatic acids.

20 The above description and examples are to be taken as illustrative only and not as limiting the scope of the invention. Any modification or variation therefrom which conforms to the spirit of the invention is intended to be included within the scope of the claims.

I claim:

1. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst.

2. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst characterized by being suitable for the synthesis of methanol from water gas.

3. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component a hydrogenating metal.

60 4. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component a hydrogenating metal oxide.

65 5. The process of producing an alcohol from an ester of a non-aromatic carboxylic acid, said alcohol corresponding in number of carbon atoms to said acid, which comprises treating with hydrogen an ester of a non-aromatic carboxylic

acid, the number of carbon atoms in said acid being greater than the number of carboxyl groups, at a temperature in excess of 200° C. and under a superatmospheric pressure in the presence of a copper-containing hydrogenation catalyst.

5

6. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a zinc-containing hydrogenation catalyst.

15

7. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component copper in combination with a hydrogenating metal oxide, said oxide being one which when exposed in a state of purity to the action of hydrogen at atmospheric pressure and at a temperature of 400° C. to 450° C. for a prolonged period of time, remains substantially in the oxide form.

20

8. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component a hydrogenating metal intimately associated with a metal oxide more acidic than the oxide of the said hydrogenating metal.

25

9. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component a hydrogenating metal oxide intimately associated with a metal oxide more acidic than the said hydrogenating metal oxide.

30

10. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a superatmospheric pressure in the presence of a hydrogenation catalyst comprising as an essential component a hydrogenating metal oxide intimately associated with chromium oxide.

35

11. The process of producing an alcohol from an ester of a non-aromatic carboxylic acid, said alcohol corresponding in number of carbon atoms to said acid, which comprises treating with hydrogen an ester of a non-aromatic carboxylic

70

75

acid, the number of carbon atoms in said acid being greater than the number of carboxyl groups, at a temperature in excess of 200° C. and under a superatmospheric pressure in the presence of 5 a hydrogenation catalyst comprising as an essential component copper oxide intimately associated with chromium oxide.

12. The process of producing an alcohol from an ester of a non-aromatic carboxylic acid, said 10 alcohol corresponding in number of carbon atoms to said acid, which comprises treating with hydrogen an ester of a non-aromatic carboxylic acid, the number of carbon atoms in said acid being greater than the number of carboxyl 15 groups, at a temperature in excess of 200° C. and under a superatmospheric pressure in the presence of a hydrogenation catalyst comprising as an essential component copper chromite.

13. The process of producing an alcohol from 20 an ester of a non-aromatic carboxylic acid, said alcohol corresponding in number of carbon atoms to said acid, which comprises treating with hydrogen an ester of a non-aromatic carboxylic acid, the number of carbon atoms in said acid 25 being greater than the number of carboxyl groups, at a temperature in excess of 200° C. and under a superatmospheric pressure in the presence of a hydrogenation catalyst comprising as an essential component zinc chromite.

14. The process of producing an alcohol from 30 an ester of an aliphatic mono-carboxylic acid, said alcohol corresponding in number of carbon atoms to said acid, which comprises treating with hydrogen an ester of an aliphatic mono- 35 carboxylic acid, said acid containing at least two carbon atoms, at a temperature in excess of 200° C. and under a superatmospheric pressure in the presence of a hydrogenation catalyst.

15. The process of producing an alcohol from 40 an ester of an aliphatic mono-carboxylic acid, said alcohol corresponding in number of carbon atoms to said acid, which comprises treating with hydrogen an ester of an aliphatic mono- 45 carboxylic acid, said acid containing at least two carbon atoms, at a temperature of between 240° C. and 400° C. and under a pressure in excess of twenty-five atmospheres in the presence of a hydrogenation catalyst.

16. The process of producing an alcohol from 50 an ester of a saturated aliphatic mono-carboxylic acid, said alcohol corresponding in number of carbon atoms to said acid, which comprises treating with hydrogen an ester of a saturated aliphatic mono-carboxylic acid, said acid containing 55 at least two carbon atoms, at a temperature of between 240° C. and 400° C. and under a pressure in excess of 25 atmospheres in the presence of a hydrogenation catalyst.

17. The process of producing an alcohol from 60 an alkyl ester of an aliphatic mono-carboxylic acid, said alcohol corresponding in number of carbon atoms to said acid, which comprises treating with hydrogen an alkyl ester of an aliphatic mono-carboxylic acid, said acid containing at 65 least two carbon atoms, at a temperature in excess of 200° C. and under a superatmospheric pressure in the presence of a hydrogenation catalyst.

18. The process of producing an alcohol from 70 an alkyl ester of an aliphatic mono-carboxylic acid, said alcohol corresponding in number of carbon atoms to said acid, which comprises treating with hydrogen an alkyl ester of an aliphatic mono-carboxylic acid, said acid containing at 75 least two carbon atoms, at a temperature of be-

tween 240° C. and 400° C. and under a pressure in excess of twenty-five atmospheres in the presence of a hydrogenation catalyst.

19. The process of producing an alcohol from 5 an ester of an aliphatic dicarboxylic acid, said alcohol corresponding in number of carbon atoms to said acid, which comprises treating with hydrogen an ester of an aliphatic dicarboxylic acid, said acid containing at least three carbon atoms, at a temperature in excess of 200° C. and under 10 a superatmospheric pressure in the presence of a hydrogenation catalyst.

20. The process of producing an alcohol from 15 an ester of adipic acid, said alcohol corresponding in number of carbon atoms to said adipic acid, 20 which comprises treating with hydrogen an ester of adipic acid at a temperature in excess of 200° C. and under a superatmospheric pressure in the presence of a hydrogenation catalyst.

21. The process of producing an alcohol from 25 an ester of an aliphatic carboxylic acid having a phenyl substituent, said alcohol corresponding in number of carbon atoms to said acid, which comprises treating with hydrogen an ester of an aliphatic carboxylic acid, said acid having a 30 phenyl substituent, at a temperature in excess of 200° C. under a superatmospheric pressure in the presence of a hydrogenation catalyst.

22. The process of producing an alcohol from 35 an ester of phenyl acetic acid, said alcohol corresponding in number of carbon atoms to said phenyl acetic acid, which comprises treating with hydrogen an ester of phenyl acetic acid at a 40 temperature in excess of 200° C. and under a superatmospheric pressure in the presence of a 35 hydrogenation catalyst.

23. The process of producing an alcohol from 45 an ester of a non-aromatic carboxylic acid, said alcohol corresponding in number of carbon atoms to said acid, which comprises treating with hydrogen an ester of a non-aromatic carboxylic 50 acid, the number of carbon atoms in said acid being greater than the number of carboxyl groups, at a temperature in excess of 200° C. but below 400° C. and under a superatmospheric pressure in 55 the presence of a hydrogenation catalyst.

24. The process of producing an alcohol from 60 an ester of a non-aromatic carboxylic acid, said alcohol corresponding in number of carbon atoms to said acid, which comprises treating with hydrogen an ester of a non-aromatic carboxylic 65 acid, the number of carbon atoms in said acid being greater than the number of carboxyl groups, at a temperature of between 240° C. and 400° C. and under a superatmospheric pressure in the presence of a hydrogenation catalyst.

25. The process of producing an alcohol from 70 an ester of a non-aromatic carboxylic acid, said alcohol corresponding in number of carbon atoms to said acid, which comprises treating with hydrogen an ester of a non-aromatic carboxylic 75 acid, the number of carbon atoms in said acid being greater than the number of carboxyl groups, at a temperature of between 240° C. and 400° C. and under a pressure in excess of twenty-five atmospheres in the presence of a hydrogenation catalyst characterized by being suitable for the synthesis of methanol from water gas.

26. The process of producing an alcohol from 80 an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, 85 90 95 75

at a temperature of between 240° C. and 400° C. and under a pressure in excess of twenty-five atmospheres in the presence of a hydrogenation catalyst comprising as an essential component a hydrogenating metal.

27. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component a hydrogenating metal oxide.

28. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. in the presence of a copper-containing hydrogenation catalyst.

29. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component copper in combination with a hydrogenating metal oxide, said oxide being one which when exposed in a state of purity to the action of hydrogen at atmospheric pressure and at a temperature of 400° C. to 450° C. for a prolonged period of time remains substantially in the oxide form.

30. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component a hydrogenating metal intimately associated with a metal oxide more acidic than the oxide of the said hydrogenating metal.

31. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component a hydrogenating metal oxide intimately associated with a metal oxide more acidic than the said hydrogenating metal oxide.

32. The process of producing an alcohol from an ester of a non-aromatic carboxylic acid, said alcohol corresponding in number of carbon atoms

to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component a hydrogenating metal oxide intimately associated with chromium oxide.

33. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component copper oxide intimately associated with chromium oxide.

34. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component copper chromite.

35. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature of between 240° C. and 400° C. and under a pressure in excess of twenty-five atmospheres in the presence of a hydrogenation catalyst comprising as an essential component zinc chromite.

36. The process of producing an alcohol from an ester of a non-aromatic carboxylic acid, said alcohol corresponding in number of carbon atoms to said acid, which comprises treating with hydrogen an ester of a non-aromatic carboxylic acid, the number of carbon atoms in said acid being greater than the number of carboxyl groups, at a temperature in excess of 200° C. and under a pressure of at least fifty atmospheres in the presence of a hydrogenation catalyst.

37. The process of producing an alcohol from an ester of an aliphatic mono-carboxylic acid, said alcohol corresponding in number of carbon atoms to said acid, which comprises treating with hydrogen an ester of an aliphatic mono-carboxylic acid, said acid containing at least two carbon atoms, at a temperature of between 240° C. and 400° C. and under a pressure in excess of twenty-five atmospheres in the presence of a hydrogenation catalyst comprising as an essential component copper chromite.

38. The process of producing an alcohol from an ester of a saturated mono-carboxylic acid, said alcohol corresponding in number of carbon atoms to said acid, which comprises treating with hydrogen an ester of a saturated aliphatic mono-carboxylic acid, said acid containing at least two carbon atoms, at a temperature of be-

tween 240° C. and 400° C. and under a pressure in excess of twenty-five atmospheres in contact with a hydrogenation catalyst comprising as an essential component copper chromite.

5 39. The process of producing an alcohol from an alkyl ester of an aliphatic mono-carboxylic acid, said alcohol corresponding in number of carbon atoms to said acid, which comprises treating with hydrogen an alkyl ester of an aliphatic 10 mono-carboxylic acid, said acid containing at least two carbon atoms, at a temperature of between 240° C. and 400° C. and under a pressure in excess of twenty-five atmospheres in contact with a hydrogenation catalyst comprising as an 15 essential component copper chromite.

40. The process of producing an alcohol from an ester of an aliphatic mono-carboxylic acid, said alcohol corresponding in number of carbon atoms to said acid, which comprises treating 20 with hydrogen an ester of an aliphatic mono-carboxylic acid, said acid containing at least two carbon atoms at a temperature of between 240° C. and 400° C. and under a pressure of at least fifty atmospheres in the presence of a 25 hydrogenation catalyst comprising as an essential component a hydrogenating metal.

41. The process of producing an alcohol from an ester of a non-aromatic carboxylic acid, said alcohol corresponding in number of carbon atoms 30 to said acid, which comprises treating with hydrogen an ester of a non-aromatic carboxylic acid, the number of carbon atoms in said acid being greater than the number of carboxyl groups, at a temperature in excess of 200° C. and under a 35 superatmospheric pressure in the presence of a hydrogenation catalyst comprising as an essential component a member of the ferrous metal group of the Periodic Table.

42. The process of producing an alcohol from an ester of a non-aromatic carboxylic acid, said alcohol corresponding in number of carbon atoms to said acid, which comprises passing a mixture 40 of hydrogen and an ester of a non-aromatic carboxylic acid, the number of carbon atoms in said acid being greater than the number of carboxyl groups, at a temperature between 240° C. and 400° C. and under a superatmospheric pressure in contact with a hydrogenation catalyst.

43. The process of producing an alcohol from an ester of a non-aromatic carboxylic acid, said alcohol corresponding in number of carbon atoms to said acid, which comprises passing a mixture 50 of hydrogen and the vapor of an ester of a non-aromatic carboxylic acid, the number of carbon atoms in said acid being greater than the number of carboxyl groups, at a temperature between 300° C. and 400° C. and under a pressure in excess of twenty-five atmospheres in contact with a hydrogenation catalyst comprising as an essential 55 component a hydrogenating metal.

44. The process of producing an alcohol from an ester of a non-aromatic carboxylic acid, said alcohol corresponding in number of carbon atoms to said acid, which comprises passing a mixture 60 of hydrogen and the vapor of an ester of a non-aromatic carboxylic acid, the number of carbon atoms in said acid being greater than the number 65 of carboxyl groups, at a temperature between 300° C. and 400° C. and under a pressure in excess of twenty-five atmospheres in contact with a hydrogenation catalyst comprising as an essential component zinc-chromite.

of carboxyl groups, at a temperature between 300° C. and 400° C. and under a pressure in excess of twenty-five atmospheres in contact with a hydrogenation catalyst comprising as an essential component a hydrogenating metal oxide.

45. The process of producing an alcohol from an ester of a non-aromatic carboxylic acid, said alcohol corresponding in number of carbon atoms to said acid, which comprises passing a mixture 10 of hydrogen and the vapor of an ester of a non-aromatic carboxylic acid, the number of carbon atoms in said acid being greater than the number of carboxyl groups, at a temperature between 300° C. and 400° C. and under a pressure in excess of twenty-five atmospheres in contact with a 15 copper-containing hydrogenation catalyst.

46. The process of producing an alcohol from an ester of a non-aromatic carboxylic acid, said alcohol corresponding in number of carbon atoms to said acid, which comprises passing a mixture 20 of hydrogen and the vapor of an ester of a non-aromatic carboxylic acid, the number of carbon atoms in said acid being greater than the number of carboxyl groups, at a temperature between 300° C. and 400° C. and under a pressure in excess of twenty-five atmospheres in contact with a 25 zinc-containing hydrogenation catalyst.

47. The process of producing an alcohol from an ester of a non-aromatic carboxylic acid, said alcohol corresponding in number of carbon atoms 30 to said acid, which comprises passing a mixture of hydrogen and the vapor of an ester of a non-aromatic carboxylic acid, the number of carbon atoms in said acid being greater than the number of carboxyl groups, at a temperature between 300° C. and 400° C. and under a pressure in excess of twenty-five atmospheres in contact with a 35 hydrogenation catalyst comprising as an essential component a hydrogenating metal oxide intimately associated with a metal oxide more acidic 40 than the said hydrogenating metal oxide.

48. The process of producing an alcohol from an ester of a non-aromatic carboxylic acid, said alcohol corresponding in number of carbon atoms to said acid, which comprises passing a mixture 45 of hydrogen and the vapor of an ester of a non-aromatic carboxylic acid, the number of carbon atoms in said acid being greater than the number of carboxyl groups, at a temperature between 300° C. and 400° C. and under a pressure in excess 50 of twenty-five atmospheres in contact with a hydrogenation catalyst comprising as an essential component a hydrogenating metal oxide intimately associated with chromium oxide.

49. The process of producing an alcohol from an ester of a non-aromatic carboxylic acid, said alcohol corresponding in number of carbon atoms to said acid, which comprises passing a mixture 55 of hydrogen and the vapor of an ester of a non-aromatic carboxylic acid, the number of carbon atoms in said acid being greater than the number of carboxyl groups, at a temperature between 300° C. and 400° C. and under a pressure in excess 60 of twenty-five atmospheres in contact with a hydrogenation catalyst comprising as an essential component zinc-chromite.

WILBUR A. LAZIER.

CERTIFICATE OF CORRECTION.

Patent No. 2,079,414.

May 4, 1937.

WILBUR A. LAZIER.

It is hereby certified that error appears in the printed specification of the above numbered patent requiring correction as follows: Page 2, first column, line 63, for the word "plate" read place; page 3, second column, line 53, for "about" read above; and that the said Letters Patent should be read with these corrections therein that the same may conform to the record of the case in the Patent Office.

Signed and sealed this 27th day of July, A. D. 1937.

Henry Van Arsdale

(Seal)

Acting Commissioner of Patents.